

# UNITED STATES PATENT OFFICE.

FREDERICK M. BECKET, OF NIAGARA FALLS, NEW YORK, ASSIGNOR TO ELECTRO METALLURGICAL COMPANY, OF NIAGARA FALLS, NEW YORK, A CORPORATION OF NEW YORK.

## ABRASIVE.

1,279,828.

Specification of Letters Patent. Patented Sept. 24, 1918.

No Drawing.

Application filed April 10, 1916. Serial No. 90,209.

To all whom it may concern:

Be it known that I, FREDERICK M. BECKET, a subject of the King of England, residing at Niagara Falls, in the county of Niagara 5 and State of New York, have invented certain new and useful Improvements in Abrasives, of which the following is a specification.

This invention relates to an abrasive substance containing as essential components iron, chromium, carbon and usually silicon, and distinguished from the heretofore known ferrochrome alloys by its composition, and by the possession to a very high degree of 10 the combined qualities of toughness, hardness, and resistance to oxidation both at low and high temperatures. In respect to this combination of qualities, the new alloy is superior to manganese steel. The alloy possesses other valuable characteristics as mentioned below.

An alloy combining toughness, hardness and resistance to oxidation to a remarkable degree contains—

|    |               |           |
|----|---------------|-----------|
| 25 | Chromium----- | 25 -30 %  |
|    | Carbon-----   | 1.5- 3 %  |
|    | Silicon-----  | 0.0- 3 %  |
|    | Iron -----    | 73 -63.5% |

30 usually with traces of manganese, sulfur, phosphorus, copper, and perhaps other elements.

To a lesser although still marked degree, this combination of qualities is found in 35 alloys outside of the range above indicated. For example, alloys containing as low as 18 per cent. and as high as 35 per cent. of chromium, the carbon and silicon being approximately as specified above, are serviceable for 40 abrasive purposes as mentioned below.

The extreme toughness and hardness of the above-mentioned alloys render them 45 highly efficient and desirable substitutes for chilled shot and crushed steel in the cutting and grinding of marble, granite and the like; and moreover, their freedom from tendency to oxidize or rust in presence of water presents the advantage that there is no liability to staining the stone. For instance, it is 50 well known that crushed steel cannot be used for marble-grinding where freedom from staining is of importance; whereas the present alloys are eminently suited for this use, in addition to being capable of much more 55 rapid cutting or grinding. The degree of

resistance to rusting is dependent in a measure upon the silicon-content of the alloy, being more strongly marked as the silicon-content is increased within the limits specified. If however the silicon-content exceeds these 60 limits a tendency to brittleness is observed.

As an illustration of resistance to oxidation at high temperatures, a cast bar of alloy containing chromium 28%, carbon 2.72%, silicon 0.40%, the balance practically 65 all iron, was exposed continuously at 1100° C. for two weeks to an oxidizing atmosphere in an electrically heated muffle furnace without undergoing appreciable oxidation, whereas a mild steel under identical conditions 70 was quickly converted into scale oxid.

Alloys within the limits above specified possess a strongly marked fibrous structure. They can be forged and machined, although with difficulty as compared with ordinary 75 steel. They can be annealed and also tempered, and in general are responsive to heat treatment, although to a materially less degree than ordinary high-carbon steels.

Among the uses to which the possession of 80 the above-mentioned properties render the new alloys particularly adapted are mentioned the following:—

(1) As an abrasive: For example the molten alloy may be poured into water in order 85 to granulate it, and the resulting granules crushed by stamping or otherwise, and graded, thereby producing irregularly shaped cutting grains or particles of approximately uniform size. The abrasive particles may be used as substitutes for chilled shot or crushed steel in the grinding and cutting of marble and granite as mentioned above, or they may be bonded by a silicate or other bond into abrasive wheels or 90 other implements, the firing being carried out under ordinary conditions in case a silicate bond is used.

(2) As a non-slipping surface in conjunction with cements, artificial stone compositions or the like.

The herein-described alloys may be prepared by various methods, as for example by melting commercial grades of high-carbon ferrochromium with the requisite proportion of steel scrap in a crucible furnace, adding if necessary silicon or ferrosilicon. The composition of the component materials being known, the proportions of such materials required to produce an alloy of any 110

desired composition is easily computed arithmetically.

I claim:

1. An abrasive material in the form of 5 irregularly shaped grains of approximately uniform size, and containing chromium 18 to 35 per cent., carbon 1.5 to 3 per cent., and silicon up to three per cent., the balance principally iron.
- 10 2. An abrasive material in the form of 15 irregularly shaped grains of approximately uniform size, and containing chromium 25 to 30 per cent., carbon 1.5 to 3 per cent., and silicon up to three per cent., the balance principally iron.
3. An abrasive wheel or other implement containing bonded grains of an alloy consisting essentially of iron, chromium and carbon in about the proportions specified.
4. An abrasive wheel or other implement 20 containing bonded grains of an alloy consisting essentially of iron, chromium, carbon and silicon in about the proportions specified.

In testimony whereof I affix my signature 25  
in presence of two witnesses.

FREDERICK M. BECKET.

Witnesses:

MARY SCAFE,  
SIDNEY OTES.

**CERTIFICATE OF CORRECTION.**

Patent No. 1,279,828.

Granted September 24, 1918, to

**FREDERICK M. BECKET.**

It is hereby certified that the State of incorporation of the assignee in the above numbered patent was erroneously given as "New York" whereas said State should have been given as "West Virginia", as shown by the records of assignments in this office; and that the said Letters Patent should be read with this correction therein that the same may conform to the record of the case in the Patent Office.

Signed and sealed this 19th day of August, A. D. 1927.

**M. J. Moore,  
Acting Commissioner of Patents.**

Seal.